

H. S. BLACKMORE.

ART OF EXTRACTING ALUMINUM AND OTHER METALS.

APPLICATION FILED JULY 31, 1907.

920,893.

Patented May 4, 1909.

Fig. 1.



Fig. 3.



WITNESSES.

Henry Willig  
Albert J. Berger

INVENTOR.

Henry Spencer Blackmore

# UNITED STATES PATENT OFFICE.

HENRY SPENCER BLACKMORE, OF MOUNT VERNON, NEW YORK.

## ART OF EXTRACTING ALUMINUM AND OTHER METALS.

No. 920,893.

Specification of Letters Patent.

Patented May 4, 1909.

Original application filed September 12, 1903, Serial No. 172,960. Divided and this application filed July 31, 1907.  
Serial No. 386,459.

*To all whom it may concern:*

Be it known that I, HENRY SPENCER BLACKMORE, a citizen of the United States, residing at Mount Vernon, in the county of 5 Westchester and State of New York, have invented certain new and useful Improvements in the Art of Extracting Aluminium or other Metals, of which the following is a specification, being a division from Serial No. 10 172,960, filed September 12th, 1903.

The object of my invention is to reduce or extract metal from a compound of the metal desired with one or more electro-negative elements, by the combined action of an electric 15 current of selective heating nature, such as an alternating or non-metal-yielding current, and an electric current of electrolytic or metal-yielding nature, such as a direct, electrolytic or similar current, in such a manner 20 that a larger yield of metal from the action of the metal-yielding current may be obtained, in shorter time, with less current, at less expense, and yielding a product of greater purity, than with processes employed hitherto. 25 With this object in view the invention consists in fusing or liquefying and maintaining fusion or liquefaction of substances containing the metal desired, by exposing the same to the action of a current of electricity of non- 30 metal-yielding nature such as an alternating current, and, while in a fused or liquefied state, liberating the metal desired by exposing the fused metal-containing substance to the action of a metal-yielding current such as 35 a direct current, with or without the presence of an augmenting reducing agent capable of uniting with the electro-negative elements liberated during action.

This process relates specifically to the reduction of aluminium from a mixture or compound consisting of aluminium combined with fluorin and oxygen by the combined fusion and electrolytic action of non-metal-yielding and metal-yielding electric currents, 40 such as alternating and direct currents, employing carbon anodes, but it is not limited thereto, as it may be applied to the reduction of many other metals without departing from the spirit of my invention. 45 In extracting the aluminium or other metal in accordance with my process as aforeslated I fuse the composition by the action of an alternating current and dissociate or reduce 50

the metal by the simultaneous action of a direct current. In this manner the constituents may be maintained in a molten condition without interrupting the action of the direct current or deteriorating the value of the same as an electrolytic agent, whereby the whole of the direct current may be expended in yielding metal instead of being utilized to a considerable extent to maintain fusion, as employed in processes hitherto. 55

The apparatus which I prefer to employ in carrying out my process is illustrated in the 60 accompanying drawing, in which,

Figure 1 is a plan or top view; Fig. 2 is a transverse vertical section; and Fig. 3 is a longitudinal vertical section.

In referring to the drawing, the letter A 70 designates a box or receptacle, preferably of cast iron, lined with a conductive substance, such as carbon B, into which project the electrodes C, C', which pass through the insulators D, D'. 75

The material is introduced into the apparatus through the openings E which are closed by the insulating covers or plugs F passing into the insulating cover X through which passes the electrodes G. 80

In the operation of the process I place in the apparatus a quantity of the substance containing the metal desired combined with fluorin and one or more non-metallic elements other than a halogen, such as aluminium with oxygen and fluorin, and fuse the same by passing an alternating current therethrough between the electrodes C, C', which heating means is independent of the electrodes G employed for electrolytic purposes. 85 I then add from time to time quantities of the composition until the interior of the apparatus has been sufficiently filled with fused material. When the substance is fused, a direct or electrolytic current is passed 90 through the mass between the electrodes G which constitute the anode and which consists preferably of carbon, and the carbon lining B which constitutes the cathode of the electrolytic circuit, the tension and intensity 95 of the current being approximately three volts and eighty-five amperes per square inch of anode surface exposed, with the temperature maintained by independent means at approximately 1800 deg. F., at which time 100 the oxygen of the substance containing alu- 105

minium, oxygen and fluorin, is liberated at the anode combining with the carbon thereof, evolving carbonic oxid gas, while metallic aluminium accumulates in the bottom of the apparatus and is withdrawn from time to time through the tap-hole H by removing the tap-hole plug I. The presence of carbon as anode augments the reduction by facilitating reduction and generating heat by union of the oxygen content therewith, thus economizing both the electrolyzing and heating currents of the electricity employed. If the electrode G consists of a material which is not acted on by the electro-negative constituent evolved at the said electrode, this augmenting action is not available. As the oxygen and aluminium are separated by electrolytic action of the direct current of such selective tension as not to affect the fluorin content, the material may be replenished from time to time by adding further increments of aluminium and oxygen in the form of aluminium oxid.

The current for heating purposes is applied independently of the electrolytic electrodes G and is passed through the substances contained in the reduction receptacle between the electrodes C, C', fusing the substances and maintaining them in a state of fusion while the electrolytic or direct current is applied through the substances between the electrodes and the carbon lining B, whereupon the electrolytic efficiency of the direct or electrolytic current may be utilized without loss. The gaseous by-products escape through the opening in the insulating covers or plugs F, shown at M, Fig. 1.

It can be seen by this method of procedure, the substance to be decomposed or electrolyzed is fused and maintained in a fused condition with the heat evolved by the resistance to the passage of the alternating or non-metal-yielding current through a fusible or fused conductor in such a manner as to heat the ingredients independent of the electrolyzing or direct current and of the electrodes through which the said current is applied.

It is well known that by passing alternating currents of electricity of high voltage and comparatively low amperage through a fusible conductor, it can be converted into heat energy, more readily with less expense and time and with more economy than can a direct or electrolytic current. It is for this reason that I prefer to term the current of electricity especially adapted to impart heat to the substances, whereby their fusion may be accomplished and maintained without decomposition, an electric current of selective heating nature in contradistinction to the more expensive direct current employed only for electrolytic purposes in the reduction of metal, after its compound has been fused or

liquefied. The present invention also has the advantage of being absolutely controlled, in that the source of the alternating, non-metal-yielding, or fusion, electric current is independent of, and separate and distinct from, the direct or electrolytic current, and each can be separately and independently controlled, so that the fusion of the electrolyte or electrolyte vehicle, and electrolysis, may be jointly accomplished. The non-metal-yielding or alternating current is disposed through the metal-containing substance in either an interrupted or continuous manner, with the direct or metal-yielding current employed at a voltage selective to the electrolytic disrupting tension of the metal-containing substance, and capable of electrically liberating the metal desired, regardless of the voltage necessary to overcome the electrical resistance of the metal-containing substances in order to fuse and maintain fusion, which is supplied by the separate non-metal-yielding or alternating current.

The prior art reveals, first, processes which depend upon fusing substances to be electrolytically reduced in melting pots by the action of heat applied external thereto, the heat of which has first to pass through the melting pot or container which brings the container to so much higher temperature than the fused contents that the melting pots become rapidly corroded and destroyed with the simultaneous contamination of the metal reduced from the molten substances in the melting pot by electrolytic action; and second, those which depend upon internal fusion such as produced by the passage of a direct current through metal-containing substances, whereby the substances are maintained in a state of fusion by the conversion of a portion of the direct current into heat energy and the metal electrolytically separated by the employment of an excess of direct current over that necessary to fuse and maintain the fusion of the substances; those depending upon the fusion of the substances by impinging a fusing heat upon the same, such as a blow-pipe flame or reverberatory furnace and electrolyzing the fused contents by an electrolytic current; and the heating of non-conductive refractory ores in a furnace, such as a reverberatory furnace until the refractory non-conductive ores become electrically conductive and then passing a direct current of electricity through the heated unfused refractory ore in sufficient volume and of sufficient intensity to fuse the same and afterward dissociating or electrolyzing the fused refractory ores by the excess of direct current over that necessarily transformed into heat energy to fuse and maintain the fusion of the refractory ores.

One of the great difficulties experienced in

the employment of internal heating processes consists in the fact that the metal-containing substances from which it is desired to separate the metal, are, in their ordinary or cold state, non-conductors of electricity. They must therefore be first heated or fused in order to render them sufficiently electrically conductive to admit of the passage of the current of electricity therethrough. This is usually accomplished by bringing the electrodes together and separating them slightly whereby a small arc between the electrodes is formed. Into this arc a small quantity of refractory ore is fed which becomes fused by the heat of the arc and as it becomes fused it forms a molten or fluid communication between the electrodes which then acts as a conductor of electricity between the electrodes as they are drawn farther and farther apart. Should, however, the electrical current be checked for a few moments from whatsoever cause, the fused substances become chilled, coating the interior of the melting pot and thus become insulators between the electrodes and the operation cannot again be started until the non-conductive strata of chilled substance is removed from between the electrodes and a new arc started re-fusing and converting the substance into a conductive condition. The prior art also reveals another form of furnace and process whereby metal-containing substances are fused, which includes the employment of a rod or bar of conductive infusible material, such as carbon, which is heated by the passage of a current of electricity therethrough of sufficient volume and intensity, which heated conductor is so disposed as to be in contact with the substance desired to be fused. It should be noted, however, in connection with this form of application of the electric heater for fusion purposes that carbon becomes a better conductor when heated than it is when cold, and therefore requires an increased flow of electric current to maintain an equivalent heating action. The prior art also reveals a species of fusion which includes the employment of a solid metal wire spiral communicating with electrical contacts, placed in a vertical position and acting as a continuous conductor heated by electrical resistance, it is obvious in the case employing a solid metal wire spiral which was placed in a vertical position, that the temperature of this spiral wire heater never reached a point at which the conductivity of the molten substances in contact therewith was a better conductor than the solid metal spiral, or in which the resistance of the molten substances was less, so that any fused substance in contact with the heated wire spiral was never maintained in a molten condition by any other means than the heat imparted by the spiral heated by electrical resistance, and the molten com-

ound was not maintained in its molten condition by the passage of electricity therethrough as employed and claimed in the present invention. The prior state of the art, however, does not reveal any means for fusing and maintaining the fusion of metal compounds whereby a direct current may be employed and wholly utilized for the purpose of yielding metal, which means covers the fusion of the metal-containing substances by the action of a non-metal-yielding electric current through a fused metal compound and electrolyzing and separating the metal from the metal compound by the action of a direct or metal-yielding current.

By the present process great advantage is obtained in maintaining fusion by passing an alternating electric current through a fused metal compound during the process of electrolysis employing a direct current, for the reason that where a direct current is used for both fusion and electrolytic purposes the electrolyte is caused to rapidly circulate between the electrodes and is thereby greatly agitated and disturbed both by this cause and from the evolution of gaseous or other products from the anode, which agitation or disturbance tends to suspend in the molten mass particles of metal electrolytically separated especially in cases where light metals like aluminium are being reduced and where the difference in gravity between the reduced metal and the electrolyte is but little. This agitation not only prevents the metal from accumulating in mass and settling from the fused electrolyte, but also causes loss from oxidation when the particles of the light metal in a heated condition come in contact with the atmosphere at the surface. This is not the case where an alternating current is employed for the reason that the circulation between the electrodes does not occur nor are there any gaseous products generated at the electrodes as in cases where a direct current is employed. The fine particles of light metal, when suspended by agitation of the electrolyte, also have a tendency to short circuit the electrolytic or direct current, occasioning loss of current and also loss of metal which may come in contact with the electro-negative constituents evolved at the anode.

The advantage of employing an electric current for fusion purposes can be seen when it is understood that the substances are fused molecularly throughout the mass instead of and in contradistinction from heat applied from an external source where the first increments of the substance are fused in juxtaposition to the heat-conveying medium while the fusion of the mass is dependent for liquefaction or fusion by heat conveyed to it through the medium of the first fused increments by convection, which, as is well known, is a slow

and unsatisfactory operation when employed in connection with refractory substances.

The employment of an alternating current for fusion purposes has the advantage 5 of preventing corrosion of apparatus which occurs when outside heating is employed, and also the difficulties as hereinbefore set forth regarding the loss of suspended metal from oxidation when reaching the surface; 10 combination with products evolved at the anode; and the settling and separation of the metal from the electrolyte and loss of current occasioned by short circuiting of the small particles of suspended metal as results 15 from the employment of a direct current for fusing and electrolytic purposes, and also prevents loss of time and attention which would be required to operate a device including a secondary metal spiral heater which 20 would require careful adjustment as to current densities and attention to prevent the metallic spiral heater from becoming fused or disintegrated whereby the heating operation would cease. Another reason why heat 25 cannot be readily communicated to a fused material from a solid secondary heater communicating therewith, is that when the heated solid comes in contact with the molten substance, there is always produced 30 in juxtaposition thereto a film of the substance which is highly heated or vaporized and which film is more or less a non-conductor of heat. This prevents the substance proper from coming in direct contact with 35 the heater and thereby interrupts or resists the imparting of the heat from the heater to the substance desired to be fused or maintained in fusion.

In the employment of the electric current 40 for heating the mass, as in the present process, however, the whole body of fused conducting substance becomes molecularly electrified and the electrical energy transformed into heat energy by the resistance thereof 45 within and throughout the body of the metal-containing compound almost immediately. Inasmuch as it requires an electric current of higher voltage to fuse and maintain fusion of metal-containing compounds than it takes to 50 liberate metal from such fused metal compounds, it can be readily seen that a further advantage is gained by employing a non-metal-yielding electric current of relatively high voltage for fusion while the more expensive direct or metal-yielding current is 55 simultaneously supplied at a lower voltage, and only of such tension that the metal desired may be liberated from its compound, thus admitting of employment of higher amperage and consequent larger metal-yielding efficiency, without over heating the compounds employed, or constituents, to a degree that the metal liberated is dissipated or volatilized by excess heat, or converted into

carbids or other metal compounds in the 65 presence of carbon or other elements which would result in loss of metal. The higher voltage fusing current can be also transmitted from source of generation to the reduction apparatus on smaller conductors or conveyers than the lower voltage and higher amperage direct current, thereby economizing cost of plant and apparatus to produce equivalent amount of metal with processes 70 depending solely upon the single direct current of electricity for the dual purpose of fusion and electrolysis for producing metal. When a direct current of electricity, capable of yielding metal from liquefied substances containing the same, is employed for the dual 75 and common purpose of accomplishing both fusion and electrolysis, it is found, for example, during the reduction of aluminium, that should the fused bath become depleted of aluminium oxid by electrolysis, that the resistance quickly rises, resulting in the burning or volatilization of the fused bath, resulting in loss, as well as electrically overloading 80 and overheating other furnaces when connected in series, to avoid which a large number of men have to be employed to rush in and re-feed or re-supply such furnaces which have become depleted of aluminium oxid, at 85 once. This is not the case in the present 90 process where the direct current can be cut off until the furnace is re-fed at leisure with aluminium oxid, the chemical bath being maintained in a state of fusion by the alternating, non-metal-yielding or heating current 95 separate and independent of the electric current capable of yielding metal. Also when a direct or metal-yielding current is 100 employed for both fusion and electrolysis the bath is not uniformly heated, but is hottest at the anodes, while the alternating, non-metal-yielding, or other heating current, as employed in this process, heats equally throughout the mass of ingredients, and thus 105 saves the anodes from combustion by overheating and produces an even fusion of the 110 ingredients.

It is well known that many metals and compounds thereof will assume a fused or molten condition when mixed or associated with each other at a lower temperature than is possible to fuse, melt, or liquefy either of the constituents individually by the action of heat, and practically applying this fact and condition I have ascertained one can mix together compounds of a metal containing fluorin, such as aluminium fluorid, and one or more non-metallic elements other than a halogen, such as aluminium oxid, and expose this mixture or composition consisting of aluminium combined with oxygen and fluorin to the action of an electric current 115 whereby the fusion of the composition and the electric dissociation of the oxid content 120 125

is accomplished at a temperature and under conditions whereby the aluminium reduced is not volatilized or dissipated, but will accumulate and settle beneath the associated ingredients, for the reason that the compounds of aluminium and oxygen and aluminium and fluorin in the fused condition are of less specific gravity than the aluminium separated, and which composition being free from other metals than aluminium avoids the production of aluminium contaminated with other metals, yielding a product of practically pure and uncontaminated form, the electrolytical dissociation being maintained at substantially the same temperature and with the same expenditure of electric current by adding to the composition more aluminium oxid from time to time to compensate for the amount electrically dissociated, thus maintaining the composition in a practically uniform condition, the dissociation being preferably carried on with the employment of an anode capable of uniting with oxygen, such as carbon.

25 The reduction of refractory metal oxids, such as aluminium oxid fused, melted, liquefied, or dissolved by the heated chemicals mixed or associated with the same, whereby they are rendered molten below their normal melting point as hereinbefore set forth, is accomplished by the direct liquefying action of the mixed or associated chemicals, or chemical bath by means other than the direct or independent action of an electric current; 30 the refractory metal oxid being added to or dissolved in the fused liquefying or solvent chemicals from time to time as the fused substance becomes depleted of the refractory oxid content by electrolytic action resulting 35 in the deposition or reduction of the metal content thereof.

The term "liquefying" employed herein is intended to imply and does imply that the metal-containing substance is reduced, transformed, or converted into a fluid condition, by solvent, fluxing, absorbing, or other action, of molten or fusible substance, or heat, with which it may be associated.

The terminology herein, referring to the electric currents, as being disposed or applied through the metal-containing substance, for the purpose of fusion and reduction, is intended to imply the passage or conveyance of the electrical currents molecularly through the mass, body, or increments of the metal-containing substances *per se*, in contradistinction to and from the passage of electricity through an independent or primary heater or conductor communicating with the ingredients to which heat may be imparted therefrom; and the term "metal-containing substance" is intended to imply a compound containing the metal in combination or a substance containing a compound 65 of the metal desired.

Having now described my invention, what I claim as new, and desire to secure by Letters Patent, is:—

1. The process of electrically producing metal, which consists in fusing a substance containing the metal desired to be produced, by the action of an alternating current disposed or applied therethrough, and liberating the desired metal therefrom by the action of a direct current. 70

2. The process of electrically producing metal, which consists in fusing a substance, containing the metal desired to be produced, by the action of an alternating current disposed or applied therethrough, and liberating the desired metal therefrom by the action of a direct current, while in the presence of a substance capable of uniting with the electro-negative constituent of the metal-containing substance to be electrolyzed. 80

3. The process of electrically producing metal from a substance containing the same, which consists in maintaining the fusion of such substance by the action of an alternating current disposed or applied therethrough, and liberating the desired metal therefrom by the action of a direct current. 90

4. The process of electrically producing metal from a substance containing the same, which consists in maintaining the fusion of such substance by the action of an alternating current disposed or applied therethrough, and liberating the desired metal therefrom by the action of a direct current, while in the presence of a substance capable of uniting with the electro-negative constituent of the metal-containing substance to be electrolyzed. 100

5. The process of electrically producing metal, which consists in maintaining the fusion of substances, containing the metal desired to be produced, by the action of a non-metal-yielding current disposed or applied therethrough, and liberating the desired metal therefrom by an electrolytic current. 105

6. The process of electrically producing metal, which consists in maintaining the fusion of a substance, containing the metal desired to be produced, by the action of a non-metal-yielding current disposed or applied therethrough, and liberating the desired metal therefrom by an electrolytic current, while in the presence of a substance capable of uniting with the electro-negative constituent of the metal-containing substance to be electrolyzed. 115

7. The process of electrically producing metal from a substance containing the metal desired to be produced, which consists in subjecting such substance to the action of an electric current of heating or non-metal-yielding nature, and an electric current of a metal-yielding nature, said heating current being disposed or applied through the sub- 125

stance independently of the electrolyzing current, whereby the electrolytic efficiency of the metal-yielding current may be utilized without loss.

5 8. The process of electrically producing metal from a substance containing the metal desired to be produced, which consists in maintaining the fusion of such substance by the action of an alternating current, disposed 10 or applied through the ingredients independently of the electrolytic electrodes, and liberating the desired metal therefrom by the action of a direct current.

15 9. The process of producing metal, which consists in maintaining fusion of a substance containing the same, by the action of a non-metal-yielding current disposed or applied therethrough, while liberating the desired metal therefrom by the action of a metal-yielding current.

20 10. The process of producing metal, which consists in exposing a metal-containing compound to the combined action of a non-metal-yielding and a metal-yielding current disposed or applied through increments of said compound.

25 11. The process of producing metal, which consists in exposing a metal-containing compound to the combined action of an alternating and a direct current disposed or applied through increments of said compound.

30 12. The process of producing metal, which consists in exposing a substance, containing the metal desired to be produced, to the combined action of an electric current of a heating nature and an electric current of an electrolyzing nature, disposed or applied through the body of said substance.

35 13. The process of producing metal, which consists in fusing a substance capable, while in a state of fusion, of liquefying metal oxids, by disposing through the same an electric current incapable of yielding metal, adding 45 to the fused substance and liquefying therein an oxid of the metal desired to be reduced, and electrolytically decomposing the liquefied metal oxid by the action of a separate or metal-yielding current.

40 14. The process of producing metal, which consists in fusing substances capable, while in a state of fusion, of liquefying metal oxids, by disposing through the same an alternating current, adding to the fused substance and 45 liquefying therein an oxid of the metal desired to be reduced, and electrolytically decomposing the liquefied metal oxid by the action of a direct current.

45 15. The process of producing metal, which consists in fusing substances capable, while in a state of fusion, of liquefying a refractory metal compound, by disposing through the same an electric current incapable of yielding metal, adding to the fused substance and

liquefying therein a refractory metal compound to be reduced, and electrolytically decomposing said liquefied compound by the action of a separate or metal-yielding current.

50 16. The process of producing metal, which consists in fusing substances capable, while in a state of fusion, of liquefying refractory metal compounds, by disposing through the same an alternating current, adding to the fused substance and liquefying therein a refractory compound of the metal desired to be reduced, and electrolytically decomposing said liquefied compound by the action of a direct current.

55 17. The process of producing metal from substances containing the same, which consists in liberating the metal by the combined action of a metal-yielding and a non-metal-yielding electric current, disposed through an electrolytic conductor containing a compound of the desired metal.

60 18. The process of producing aluminium from substances containing the same, which consists in liberating the aluminium by the combined action of a metal-yielding and a non-metal-yielding electric current, disposed through an electrolytic conductor containing a compound of the desired metal.

65 19. The process of producing aluminium, which consists in fusing substances capable, while in a state of fusion, of liquefying aluminium compounds, by disposing through the same an electric current incapable of yielding metal, adding to the fused substance and liquefying therein the aluminium compound to be reduced, and electrolytically decomposing said liquefied compound by the action of a separate or metal-yielding current.

70 20. The process of producing aluminium, which consists in fusing substances capable, while in a state of fusion, of liquefying aluminium compounds, by disposing through the same an alternating current, adding to the fused substance and liquefying therein the aluminium compound to be reduced, and electrolytically decomposing the liquefied aluminium compound by the action of a direct current.

75 21. The process of producing aluminium, which consists in fusing substances capable, while in the state of fusion, of liquefying aluminium oxid, by disposing through the same an electric current incapable of yielding metal, adding to the fused substance and liquefying therein aluminium oxid, and electrolytically decomposing said liquefied oxid by the action of a separate or metal-yielding current.

80 22. The process of producing aluminium, which consists in fusing substances capable, while in a state of fusion, of liquefying aluminium oxid, by disposing through the same

an alternating current, adding to the fused substance and liquefying therein aluminium oxid, and electrolytically decomposing said liquefied oxid by the action of a direct current.

23. The process of producing metal from substances containing the same, which consists in liberating the metal by the combined and simultaneous action of a metal-yielding and a non-metal-yielding electric current, disposed through an electrolytic conductor containing a compound of the desired metal.

24. The process of producing aluminium from substances containing the same, which consists in liberating the aluminium by the combined and simultaneous action of a metal-yielding and a non-metal-yielding electric current, disposed through an electrolytic conductor containing a compound of the desired metal.

25. The process of producing metal from substances containing the same, which consists in liberating the metal by the combined action of a metal-yielding and a non-metal-yielding electric current, disposed through a fused electrolytic conductor containing a compound of the desired metal dissolved therein.

30 26. The process of producing aluminium from substances containing the same, which consists in liberating the aluminium by the combined action of a metal-yielding and a non-metal-yielding electric current, disposed through a fused electrolytic conductor containing a compound of the desired metal dissolved therein.

35 27. The process of producing metal from substances containing the same, which consists in liberating the metal by the combined action of a direct and an alternating electric current, disposed through an electrolytic conductor containing a compound of the desired metal.

45 28. The process of producing aluminium from substances containing the same, which consists in liberating the aluminium by the combined action of a direct and an alternating electric current, disposed through an electrolytic conductor containing a compound of the desired metal.

55 29. The process of producing metal from substances containing the same, which consists in liberating the metal by the combined and simultaneous action of a direct and an alternating electric current, disposed through an electrolytic conductor containing a compound of the desired metal.

60 30. The process of producing aluminium from substances containing the same, which consists in liberating the aluminium by the combined and simultaneous action of a direct and an alternating electric current, dis-

posed through an electrolytic conductor containing a compound of the desired metal.

31. The process of producing metal from substances containing the same, which consists in liberating the metal by the combined action of a direct and an alternating electric current, disposed through a fused electrolytic conductor containing a compound of the desired metal dissolved therein.

32. The process of producing aluminium from substances containing the same, which consists in liberating the aluminium by the combined action of a direct and an alternating electric current, disposed through a fused electrolytic conductor containing a compound of the desired metal dissolved therein.

33. The process of electrically decomposing or transforming chemical compounds, which consists in fusing such compounds by the action of a non-metal-yielding current, disposed or applied through the same, and producing the desired product by the action of an electrolytic current.

34. The process of electrically decomposing or transforming chemical compounds, which consists in fusing such compounds by the action of an alternating current disposed or applied through the same, and producing the desired product by the action of a direct current.

35. The process of electrically decomposing or transforming chemical compounds, which consists in fusing such compounds by the action of a non-metal-yielding current, disposed or applied through the same, and producing the desired product by the simultaneous action of an electrolytic current.

36. The process of electrically decomposing or transforming chemical compounds, which consists in fusing such compounds by the action of an alternating current disposed or applied through the same, and producing the desired product by the simultaneous action of a direct current.

37. The process of electrically decomposing or transforming chemical compounds, which consists in fusing such compounds by the action of a non-metal-yielding current, disposed or applied through the same, and producing the desired product by the action of an electrolytic current and chemical affinity.

38. The process of electrically decomposing or transforming chemical compounds, which consists in fusing such compounds by the action of an alternating current disposed or applied through the same, and producing the desired product by the action of a direct current and chemical affinity.

39. The process of electrically decomposing or transforming chemical compounds, which consists in fusing such compounds by the action of a non-metal-yielding current,

disposed or applied through the same, and producing the desired product by the simultaneous action of an electrolytic current and chemical affinity.

40. The process of electrically decomposing or transforming chemical compounds, which consists in fusing such compounds by the action of an alternating current disposed or applied through the same, and producing

the desired product by the simultaneous 10 action of a direct current and chemical affinity.

In testimony whereof I affix my signature in presence of two witnesses.

HENRY SPENCER BLACKMORE.

Witnesses:

H. N. JENKINS,

J. R. NOTTINGHAM.